



US008709555B2

(12) **United States Patent**  
**Pal et al.**

(10) **Patent No.:** **US 8,709,555 B2**  
(b5) **Date of Patent:** **Apr. 29, 2014**

- (54) **MEDIA USED IN DIGITAL HIGH SPEED INKJET WEB PRESS PRINTING**
- (75) Inventors: **Lokendra Pal**, San Diego, CA (US); **Jason Swei**, San Diego, CA (US); **Glenn T. Gentile**, San Diego, CA (US); **Sandeep K. Bangaru**, San Diego, CA (US)
- (73) Assignee: **Hewlett-Packard Development Company, L.P.**, Houston, TX (US)
- (\*) Notice: Subject to any disclaimer, the term of this patent is extended or adjusted under 35 U.S.C. 154(b) by 0 days.
- (21) Appl. No.: **14/113,199**
- (22) PCT Filed: **Apr. 28, 2011**
- (86) PCT No.: **PCT/US2011/034403**  
§ 371 (c)(1),  
(2), (4) Date: **Oct. 21, 2013**
- (87) PCT Pub. No.: **WO2012/148405**  
PCT Pub. Date: **Nov. 1, 2012**

(65) **Prior Publication Data**

US 2014/0044896 A1 Feb. 13, 2014

- (51) **Int. Cl.**
- B41M 5/00** (2006.01)  
**B41M 5/50** (2006.01)  
**B41M 5/52** (2006.01)  
**D21H 11/04** (2006.01)  
**D21H 11/12** (2006.01)  
**D21H 13/06** (2006.01)  
**D21H 17/29** (2006.01)  
**D21H 21/20** (2006.01)  
**D21H 25/14** (2006.01)
- (52) **U.S. Cl.**
- CPC ..... **B41M 5/502** (2013.01); **B41M 5/504** (2013.01); **B41M 5/508** (2013.01); **B41M 5/5218** (2013.01); **D21H 11/04** (2013.01); **D21H 11/12** (2013.01); **D21H 13/06** (2013.01); **D21H 17/29** (2013.01); **D21H 21/20** (2013.01); **D21H 25/14** (2013.01)

USPC ..... **428/32.21**; 428/32.22; 162/135; 162/136; 162/141; 162/147; 162/149; 162/158; 162/175; 162/189; 162/231

- (58) **Field of Classification Search**
- CPC ..... B41M 5/502; B41M 5/504; B41M 5/508; B41M 5/5218; D21H 11/04; D21H 11/12; D21H 13/06; D21H 17/29; D21H 21/20; D21H 25/14
- USPC ..... 428/32.21, 32.22; 162/135, 136, 141, 162/147, 149, 158, 175, 189, 231
- See application file for complete search history.

(56) **References Cited**

U.S. PATENT DOCUMENTS

6,277,477 B1 \* 8/2001 Tracy et al. ..... 428/32.23  
6,287,743 B1 9/2001 Oakland et al.

(Continued)

OTHER PUBLICATIONS

Aidun, Cyrus K., Final Report Improving Paper Machine Efficiency Through On-Line Control of Stock Delivery, Headbox and Forming Hydrodynamics, Award No. De-FC36-99GO10416, Institute of Paper Science and Technology at Georgia Tech., Atlanta, GA, 2006, 35 pages. (from <<http://www1.eere.energy.gov/industry/forest/pdfs/aidun.pdf>>).

(Continued)

*Primary Examiner* — Betelhem Shewareged

(57) **ABSTRACT**

A media for digital high speed inkjet web press printing has a CD residual tensile energy absorption index greater than 300 J/Kg. The media includes a paper base having a MD/CD tensile stiffness index ratio of less than 2.0 and a tensile energy absorption index of greater than 500 J/Kg. The paper base includes a mixture of fibers having a softwood fiber to hardwood fiber ratio within a range of 3 to 7 to 7 to 1, an internal starch having a cationic starch to fiber ratio greater than 1.0%, and a filler within a range of about 1.0% to about 12.0% of paper base weight. The media further includes an image receiving coating on a side of the paper base.

**15 Claims, 2 Drawing Sheets**

200



(56)

**References Cited****U.S. PATENT DOCUMENTS**

- 6,805,929 B2 \* 10/2004 Koga et al. .... 428/32.11  
7,037,457 B2 5/2006 Seidel et al.  
7,160,419 B2 1/2007 Suzuki et al.  
2003/0087208 A1 5/2003 Bourdelais et al.  
2004/0149412 A1 8/2004 Tammi et al.  
2004/0200593 A1 10/2004 Koskinen et al.  
2004/0258857 A1 12/2004 Dagan et al.  
2008/0118676 A1 5/2008 Yamamoto et al.  
2009/0035478 A1 2/2009 Zhou et al.  
2009/0061332 A1 3/2009 Tamagawa et al.  
2010/0043991 A1 2/2010 Huang et al.  
2011/0171385 A1 \* 7/2011 Pal et al. .... 427/256

**OTHER PUBLICATIONS**

Aidun, Cyrus K., Improving Paper Machine Efficiency Through On-Line Control of Stock Delivery, Headbox and Forming Hydrodynamics, Award No. De-FC36-99GO10416, Institute of Paper Science and

Technology at Georgia Tech., Atlanta, GA, Apr. 6, 2006, 36 View graphs. (from < <http://www1.eere.energy.gov/industry/forest/pdfs/aidun.pdf> >).

Properties of Paper, 15 pages (from < <http://www.paperonweb.com/paperpro.htm> >), Nov. 23, 2010.

Better Quality and Runnability through Fiber Orientation Optimization, copyright 2010 METSO, 2 pages (from < <http://www.metso.com/pulpandpaper/MPwArticles.nsf/WebWID/WTB-100121-2256F-B9DEB?OpenDocument> >).

Gentile, Louis et al., Optimizing Press Section and Paper Machine Performance, Apr. 2006, 24 pages (from < <http://www.tappi.org/Bookstore/Technical-Papers/Conference-Papers/2006/06PM/Optimizing-Press-Section-and-Paper-Machine-Performance-2006-Papermakers-Conference.aspx> >).

International Search Report (ISR) and Written Opinion of from the International Searching Authority (ISA/KR) for counterpart PCT patent application No. PCT/US2011/034403, dated Jan. 5, 2012 (8 pages).

\* cited by examiner



*FIG. 1A*



*FIG. 1B*



FIG. 2

## 1

**MEDIA USED IN DIGITAL HIGH SPEED  
INKJET WEB PRESS PRINTING**CROSS-REFERENCE TO RELATED  
APPLICATIONS

N/A

STATEMENT REGARDING FEDERALLY  
SPONSORED RESEARCH OR DEVELOPMENT

N/A

## BACKGROUND

There are a variety of methods for commercial high speed printing to produce large quantities of print material, such as books, magazines, newsprints, and brochures. In the past, traditional analog printers, such as web fed offset and gravure contact printers, were the most common type of printers for such commercial applications. In recent years, digital web fed high speed inkjet non-contact printers have become more prevalent due to 100% variable print content and multi-color printing at a relatively low cost to consumers.

Paper media for these more traditional types of web-fed offset or gravure printers have a high ratio of machine direction (MD) to cross-machine direction (CD) tensile stiffness that may be achieved during paper manufacturing. The high MD/CD tensile stiffness ratio means the print media can withstand the tension from being pulled tight around rollers that move the web in the machine direction at high speed in the press during printing. Paper media typically used for these more traditional analog printers can perform somewhat acceptably on high speed web fed inkjet (non-contact) printing devices.

## BRIEF DESCRIPTION OF THE DRAWINGS

Various features of examples in accordance with the principles described herein may be more readily understood with reference to the following detailed description taken in conjunction with the accompanying drawings, where like reference numerals designate like structural elements, and in which:

FIGS. 1A and 1B illustrate side views of media according to examples in accordance with the principles described herein.

FIG. 2 illustrates a flow chart of a method of making media according to an example in accordance with the principles described herein.

Certain examples have other features that are one of in addition to and in lieu of the features illustrated in the above-referenced figures. These and other features are detailed below with reference to the preceding drawings.

## DETAILED DESCRIPTION

While paper media typically used for more traditional analog printers can perform somewhat acceptably on high speed web fed inkjet (non-contact) printing devices, such paper media are subject to problems relating to one or more of cockle, curl, wrinkle, crease and mis-registration and other similar problems, which can detrimentally impact productivity, product quality and cost. For example, inkjet printing has a much higher moisture level than offset and gravure printing due to the colored pigments of the inkjet ink being applied to the paper media using a generally water based liquid vehicle.

## 2

Therefore, examples in accordance with the principles described herein are directed to a media that is more useful in digital high speed inkjet web press printing. The media according to the principles herein exhibits improved runnability during printing and finishing. The media is a light weight, coated, paper-based media in that the media comprises a paper base and a coating on one or both surfaces of the paper base that facilitates image formation on the media. The paper base has a machine direction/cross-machine direction (MD/CD) tensile stiffness index (TSI) ratio of less than 2.0 and a tensile energy absorption (TEA) index of greater than 500 J/Kg (TEA per basis weight) in each of the machine direction (MD) and the cross-machine direction (CD). Moreover, the media has a CD residual tensile energy absorption index greater than 300 J/Kg.

The low MD/CD TSI ratio means there are more random fiber orientations in the paper base at the expense of aligned fibers in the MD. More random fiber orientations mean more CD tensile stiffness that facilitates less CD (non-uniform) hygro-expansion of paper base fibers. Non-uniform hygro-expansion appears to be related to cockle and mis-registration issues, for example. Cockle refers to a small scale expansion in paper fiber width when wetted with water, for example from water-based inkjet inks. The low MD/CD TSI ratio was achieved mainly by reducing a difference between jetting speed and forming wire speed during paper manufacturing. The high TEA index (in both MD and CD) was achieved by increasing a ratio of cationic starch to fiber in the paper base. The high TEA index values mean a stronger media that has improved runnability during printing and during finishing with reduced (and in some examples, minimized) web breaks, cockling, wrinkling and creasing, for example. The media according to the principles described herein may provide one or more of excellent print quality, improved runnability during printing and finishing (one or both of inline and offline), and improved sheet cut quality for digital high speed inkjet web press production.

The paper base of the media according to the principles described herein comprises a mixture of softwood fibers and hardwood fibers. A ratio of softwood to hardwood fibers in the mixture is within a range of about 3 to about 7 to about 7 to about 1 (i.e., 3:7 to 7:1). In some examples, the softwood to hardwood ratio is a minimum of 3:7 and a maximum of 7:1. Moreover, the paper base comprises internal starch and inorganic filler. The internal starch includes, but is not limited to, a cationic starch provided in a ratio of cationic starch to fiber that is greater than 1.0%. The filler is provided in an amount sufficient to achieve ash content in a range of about 1.0% to about 12.0% of paper base weight.

In some examples, the paper base further comprises one or more agents and additives in a combined amount within a range of about 0.0075% to about 9.00% of fiber weight. For example, the paper base may further comprise internal sizing, one or more of a biocide, a preservative, a bleaching agent, one or both of a retention aid and a drainage aid, an optical brightening agent (OBA) and other functional additives and operational additives including, but not limited to dyes, defoaming agents, buffering agents, and pitch control agents, for example.

Further, the paper base may be surface treated or coated to improve holdout and fixing of an inkjet ink image on the surface of the media. The surface treatment solution or coating on the paper base is an image receiving layer that may be applied on one side or on both opposite sides of the paper base. The image receiving layer is compatible with water-based or solvent-based inkjet inks and therefore, also may be referred to herein as an ink receiving layer composition, sur-

face treatment solution or coating. Such ink receiving compositions may include ink fixing agents, including but not limited to, a divalent metallic salt, a multivalent metallic salt (e.g., of calcium, magnesium or aluminum) and a combination of any these salts; and surface sizing additives (e.g., starch, fillers, and polymeric sizing agents). In addition, the ink receiving compositions may include one or more of pigments (e.g., clay and silica); binders (e.g., latex and polyvinyl alcohol); and other additives, for example, in a variety of combinations. Moreover, the inkjet inks that form images on the media may be dye-based or pigment-based carried and delivered to the paper media using water-based chemical solutions.

In some examples, the media (i.e., coated with the image receiving layer) used in digital high speed inkjet web press printing, as described herein, has a MD/CD TSI ratio of equal to or less than 1.9. The media further has a CD tensile energy absorption index of greater than 800 J/Kg.

As used herein, the article 'a' is intended to have its ordinary meaning in the patent arts, namely 'one or more'. For example, 'a filler' generally means one or more fillers and as such, 'the filler' means 'the filler(s)' herein. The phrase 'at least' as used herein means that the number may be equal to or greater than the number recited. The term 'about' as used herein means that the number recited may differ by plus or minus 10%, for example, 'about 5' means a range of 4.5 to 5.5. The term 'between' when used in conjunction with two numbers such as, for example, 'between about 2 and about 50' includes both of the numbers recited. Any ranges of values provided herein include values and ranges within or between the provided ranges. The term 'substantially' as used herein means a majority, or almost all, or all, or an amount with a range of about 51% to 100%, for example. Also, any reference herein to 'top', 'bottom', 'upper', 'lower', 'up', 'down', 'back', 'front', 'left' or 'right' is not intended to be a limitation herein. The designations 'first' and 'second' are used herein for the purpose of distinguishing between items, such as 'first side' and 'second side', and are not intended to imply any sequence, order or importance to one item over another item or any order of operation, unless otherwise indicated. Moreover, examples herein are intended to be illustrative only and are presented for discussion purposes and not by way of limitation.

In accordance with the principles described herein, the media used in digital high speed inkjet web press printing is a light weight, coated, porous media that has a low MD/CD TSI ratio of less than 2.0 to reduce CD hygro-expansion and cockle. The media further has a high TEA index of greater than 600 J/Kg to improve web press runnability and finisher runnability, including one or more of inline, near-line and offline finishing. As such, in digital high speed inkjet web press printing and finishing, the media exhibits acceptable sheet cut quality, for example clean edges with reduced fraying, fiber feathering or other general unevenness, and with reduced tendency to crease, cockle, wrinkle, or suffer web breaks. The low MD/CD TSI ratio of the media is achieved in part by increasing random fiber orientations in the paper base at the expense of fibers oriented in the machine direction (MD) when a paper web is formed. Increasing the random fiber orientations is described further below with respect to a method of making such media. In addition, a concomitant loss in MD TSI (due to less fiber orientation in MD) is compensated by increasing a level of cationic starch in the fiber furnish. In particular, increasing a cationic starch to fiber ratio of the paper base provides or facilitates the high TEA index characteristics of the media according to the principles described herein.

Moreover, the low MD/CD TSI ratio of less than 2.0 and high TEA index of greater than 600 J/Kg for the media are achieved in part by using a paper base that comprises a fiber mixture of softwood fibers and hardwood fibers in a softwood to hardwood fiber ratio that is within a range of about 3 to about 7 to about 7 to about 1, for example. In some examples, the softwood to hardwood fiber ratio is within a range of 3 to 6 to 6 to 1, or 3 to 5 to 5 to 1, or 3 to 4 to 4 to 1, 3 to 3 to 3 to 1, or any range in between these ranges, for example about 3 to about 7 to about 3 to about 1. In some examples, the softwood to hardwood fiber ratio is within a range of 3 to 3.5 to 3 to 4, or may be 1 to about 2. In another example, the softwood to hardwood fiber ratio is within a range of about 3 to about 1 to about 2 to about 1, or about 3 to about 7 to about 1 to about 1. Fibers from hardwood pulps have a shorter fiber structure and reduced strength with refining than softwood fibers. Therefore, a higher amount of softwood fiber is added to the fiber mixture or pulp to facilitate improved tensile stiffness and TEA. In some examples, the fiber mixture comprises a minimum of 30% softwood fibers. As such, the paper base of the media herein has a TEA Index that is not less than 500 J/Kg, or not less than 600 J/Kg, or not less than 700 J/Kg, for example.

Examples of softwoods useful for the fiber mixture include, but are not limited to, northern softwoods and southern softwoods, such as White Spruce and Pine from North America. Examples of hardwoods useful for the fiber mixture include, but are not limited to, southern hardwoods and northern hardwoods, such as Birch, Maple, and Aspen from North America. The fiber mixture of the paper base may further include non-wood fibers (e.g., one or more of bamboo, bagasse and straw), and recycled fiber (e.g., pre- and post-consumer fiber). The fibers may be included in the form of chemical pulp, mechanical pulp, or a hybrid pulp including, but not limited to, thermal mechanical pulp, chemical mechanical pulp, and Chemi-Thermo-Mechanical (CTMP) pulp, or a combination of any of these, for example. Examples of chemical pulps used in the fiber mixture include, but are not limited to, one or more kraft pulps and sulfite pulps, each of which may or may not be bleached. Bleached pulp is used to avoid possible brownish tint typically found in unbleached pulp.

In some examples, recycled pulp, mechanical pulp, hybrid pulp and non-wood fiber pulp each independently may be included in the fiber mixture in an amount (of total fiber weight) within a range of 0% to about 30%, or about 5% to about 30%, or about 10% to about 25%, or about 15% to about 20%, for example. In some examples, up to about 15% of the fiber mixture is recycled pulp. In some examples, up to about 10% of the fiber mixture is mechanical pulp or a hybrid pulp. In some examples, the fiber mixture may include a range of about 25% to about 35% softwood chemical pulp, a range of about 20% to about 30% hardwood chemical pulp, and a combined amount in a range of about 40% to about 50% mechanical pulp, hybrid pulp and recycled pulp, such that a total amount of softwood in the fiber mixture is at least 30%. For example, the fiber mixture may include about 30% of softwood chemical pulp, about 25% hardwood chemical pulp, about 18% hybrid pulp and about 25% recycled pulp, such that a total amount of softwood in the fiber mixture is greater than 30%.

The paper base further comprises internal starch and inorganic filler. These internal agents are added to the fiber mixture or pulp stock before it is converted into a paper web (i.e., the paper base). The internal starch improves dry strength, and cationic starch may further act as a retention aid, for example. The internal starch includes a cationic starch and

may further include one or more of anionic, cross-linked, liquid or dry pre gel, nonionic and amphoteric starch. The internal starch may be corn-based or potato-based, for example. The internal starch is provided in an amount that has a cationic starch to fiber ratio that is greater than 1.0%. In some examples, the ratio of cationic starch to fiber is equal to or greater than about 1.10%. In some examples, the cationic starch to fiber ratio is within a range of greater than 1.0% to about 5.0%, or in some examples, a minimum of 1.10% and a maximum of 5.0%. In some examples, the total internal starch (cationic and other types of starch) is provided in an amount within a range of greater than 1.0% to about 11.0% of the fiber weight. In some examples, the amount of the total internal starch is within a range of about 1.10% and about 11.0% of the fiber weight, or about 1.5% and about 11.0% of the fiber weight, or about 1.5% and about 10.0% of the fiber weight, or about 2.0% and about 11.0% of the fiber weight, or about 3.0% and about 11.0% of the fiber weight. Examples of starch include, but are not limited to, CHARGEMASTER® L335 Cationic Starch from GPC, Muscatine, Iowa, USA; Apollo® Cationic Corn Starch, Astro X® Cationic Potato Starch, Pen-cat® Cationic Corn Starch, and Topcat® Cationic Additive from Penford Products Company, Cedar Rapids, Iowa, USA; and STA-LOK® 120, 140, 160, 180 Cationic Waxy Starch, STA-LOK® 156, 182 Amphoteric Waxy Corn Starch, and STA-LOK® 300, 310, 330 Cationic Dent Corn Starch from TATE and LYLE, Decatur, Ill., USA (formerly A E Staley).

The inorganic filler substantially controls some physical properties of the paper base, for example. Particles of the filler fill in the void spaces of the fiber network and substantially result in one or more of a denser, smoother, and brighter paper base than without filler. However, less filler may be better for strength for example. Examples of fillers that may be incorporated into the fiber mixture of the paper base include, but are not limited to, ground calcium carbonate (GCC), precipitated calcium carbonate (PCC), titanium dioxide, clays and talc and combinations of any of the above. In some examples, the paper base comprises an amount by dry weight of filler (measured as ash content %) within a range of about 1.0% to about 12% of the paper base weight. In some examples, the amount of filler (ash content %) in the paper base ranges from about 1.0% to about 10.0%, or about 3.0% to about 10.0%, or about 5.0% to about 10.0%, or about 7.0% to about 10.0% by paper base weight. In some examples, the filler is provided in an amount sufficient to achieve less than about 12% ash content. Examples of filler include, but are not limited to, Magfil® PCC from Specialty Minerals, Inc. of Bethlehem, Pa., USA, or Omyafil® GCC from Omya North America.

In some examples, the paper base further comprises agents and additives that provide functional and operational benefits. These agents and additives also may be added to the fiber mixture or pulp stock before it is converted to the paper web. For example, an internal sizing may be provided in the fiber mixture of the paper base in an amount greater than 0.01% of the fiber weight to improve water resistance properties. For example, more internal sizing may lessen ink-water interaction with the fibers in the paper base. In some examples, internal sizing may be included in an amount within a range of about 0.015% and about 1.00% of the fiber weight. Examples of internal sizing agents include, but are not limited to, one or more of fatty acids, alkyl ketene dimer (AKD) emulsification products, alkenyl acid anhydride emulsification products, alkylsuccinic acid anhydride (ASA) emulsification products, and rosin derivatives. Some examples of commercially available ASA and AKD include, but are not limited to, Nalco 7542 ASA from Nalco Company, IL, USA and AKD 2030 from BASF, and Hercon 195 AKD from Hercules Inc. USA.

In some examples, the paper base may further comprise from about 0.01% to about 5.00% by fiber weight of one or more of a biocide, a bleaching agent and a preservative (herein collectively 'bleach/biocide'). Some examples of commercially available biocides include, but are not limited to, Busan®1124, 1130, 1210, 1223 from Buckman Laboratories, Memphis, Tenn., USA and Spectrum™ XD3899 micro-biocide from Ashland Inc., Covington, Ky., USA. In some examples, the amount of bleach/biocide is about 1% by fiber weight. In some examples, the paper base may further comprise about 0.05% to about 2.00% by fiber weight of one or both of a retention aid and a drainage aid (herein collectively 'retention/drainage' aid). Examples of retention/drainage aids include, but are not limited to, one or more of a polyacrylamide, polyaluminum chloride, silica-type micro-particles, a flocculant and a dispersant. In some examples, about 0.10% to about 0.30% by fiber weight of a retention/drainage aid is included in the paper base. In some examples, the paper base may further comprise an optical brightening agent (OBA) to control color, for example, in an amount within a range of about 0.0075% to about 0.25% by fiber weight. In some examples, about 0.04% to about 0.06% by fiber weight of OBA is included in the paper base. Other agents and additives including, but not limited to, dyes, defoaming agents, buffering agents and pitch control agents may be included in the fiber mixture of the paper base in some examples. These other agents and additives may be included in a combined amount within a range of about 0.0075% to about 9.0% by fiber weight, or about 0.08% to about 8.5%, or about 0.10% to about 6.0%, or about 0.50% to about 5.0%. In some examples, the combined amount of these other agents and additives in the paper base is within a range of about 1.0% to about 2.0% by fiber weight.

In some examples, the paper base may receive one or more layers or coatings (e.g., a surface sizing) to the paper web surface in a paper machine during paper manufacture. These layers or coatings facilitate one or more of smoothness, whiteness, gloss, porosity, and opacity, for example, of the paper web. These coatings are intermediate coatings that are separate and distinguishable from the image receiving coating layer further described herein. As such, the paper base may be uncoated (e.g., no surface sizing), or coated with intermediate coatings (e.g., of surface sizing), as mentioned herein, depending on the example, before the image receiving surface treatment or coating layer is applied.

In some examples, the paper base of the media has a basis weight within a range of about 30 grams per square meter (gsm) to about 74 gsm. In some examples, the basis weight of the paper base is within a range of about 35 gsm to about 74 gsm, or about 40 gsm to about 74 gsm, or about 45 gsm to about 74 gsm, or about 50 gsm to about 74 gsm, or about 60 gsm to about 74 gsm. In some examples, the basis weight of the paper base of the media is about 50 gsm to about 60 gsm.

According to the principles described herein, the media includes an image receiving layer (i.e., surface treatment or coating) on one or both sides of the paper base of the media. FIG. 1A illustrates an example of the media 100) with an image receiving layer 120) on one side of the paper base 110); and FIG. 1B illustrates an example of the media 100) with an image receiving layer 120) on both sides of the paper base 110), each in accordance to the principles described herein. The image receiving layer 120) comprises an image receiving composition capable of receiving and retaining an inkjet ink imaging material applied in a pattern (or image) to the layer. The image receiving layer 120) is an outermost layer on the paper base 110). The inkjet ink may be water-based or solvent-based and includes either dyes or pigments for color,

depending on the particular inkjet ink. In some examples, the image receiving layer **120**) may facilitate relatively improved bleed and dry time of the inks that are applied thereto. There are a variety of image receiving compositions that may be used for the image receiving layer **120**) on the paper base **110** of the media **100**) according to the principles described herein.

In some examples, the image receiving composition comprises ink fixing agents including, but not limited to, divalent or multivalent metallic salts (e.g., a chloride, a bromide, a nitrate or an acetate of calcium, magnesium or aluminum or a combination of any of these); one or both of inorganic pigment fillers (e.g., clay, carbonates, silica gels, and fumed silica) and organic pigment fillers (e.g., polystyrene and polyacrylates); one or both of a water-based binder and a water dispersible binder (e.g., latex, polyvinyl alcohol (PVA), starch, styrene-butadiene or acrylates); and one or more of a variety of additives. For example, other additives including, but not limited to, one or more of surface sizing agents, wetting agents, de-foaming agents, anti-foaming agents and dispersing agents also may be incorporated into the image receiving layer.

In some examples, a basis weight of the image receiving coating on the paper base is within a range of about 1 gsm to about 15 gsm. The coating basis weight is a total of the coating basis weight on one or on both sides of the paper base. In some examples, the total coating basis weight on the paper base is within a range of about 2 gsm to about 15 gsm, or about 4 gsm to about 15 gsm, or about 6 gsm to about 15 gsm, or about 8 gsm to about 15 gsm, or about 10 gsm to about 15 gsm, or for example, a total coating basis weight of about 13 gsm.

As such, the media according to the principles described herein is light weight, for example having a basis weight within a range of about 31 gsm to about 75 gsm. In some examples, the basis weight of the media is within a range of about 35 gsm to about 75 gsm, or about 40 gsm to about 75 gsm, or about 45 gsm to about 75 gsm, or about 55 gsm to about 75 gsm, or about 60 gsm to about 70 gsm. In some examples, the basis weight of the media is less than 75 gsm, for example about 70 gsm, or about 65 gsm.

A method of making media used in digital high speed inkjet web press printing is also provided. FIG. 2 illustrates a flow chart of a method **200**) of making such media according to an example of the principles described herein. The method **200**) of making comprises forming **210**) a pulp stock that comprises a fiber mixture of refined cellulose fibers and non-fibrous functional and operational additives and agents. For example, the cellulose fiber mixture includes softwood fibers and hardwood fibers in a softwood:hardwood ratio that is within a range of about 3:7 to about 7:1. In some examples, non-wood fiber may be included also. The softwood, the hardwood and the non-wood fibers are provided as one or more of recycled pulp, chemical pulp, mechanical pulp, and hybrid pulp, for example. In some examples, the fiber mixture includes about 50% to about 60% chemical pulp. In some examples, about 15% to about 30% recycled pulp may be included in the fiber mixture. In other examples, about 10% to about 20% of one or both mechanical pulp and hybrid pulp may be included in the fiber mixture either in addition to or in lieu of the recycled pulp. In the above examples, at least 30% of the pulp in the fiber mixture is softwood. The fiber mixture is substantially the same as that described above for the paper base of the media according to the principles herein.

In some examples, wood chips may be pressure-cooked with a mixture of water and chemicals in a digester to form a pulp. In fiber mixtures that include non-wood fibers, non-

wood chips are cooked in a separate digester with respective chemicals and then added to the wood pulp mixture. In other examples, commercially available virgin softwood and hardwood fibers may be used. The pulp is washed, cleaned and in some examples, bleached, then refined in a beater or refiner using one or both of chemical and mechanical refining. The non-fibrous functional and operational additives and agents are added and mixed with the pulp to form the pulp stock (i.e., fiber furnish). Such additives and agents include internal starch and inorganic filler, as well as other additives and agents, (e.g., internal sizing, OBA etc.) described above for the examples of the paper base of the media.

In some examples, the softwood to hardwood fiber ratio and the amounts of filler and internal starch are substantially equivalent to the amounts described above for the examples of the paper base of the media. In some examples, the amounts of other agents and additives are also substantially equivalent to the amounts described above for the examples of the paper base of the media.

The method **200**) of making media further comprises jetting **220**) the pulp stock onto a moving wire screen of a paper making machine at a jet-to-wire speed ratio of between about 0.95 and about 1.05 to form an initial paper web. The jet-to-wire speed ratio is dependent on the paper making machine used, and more particularly, the machine components or configuration used, e.g., headbox, slice, or forming board, etc. As the pulp travels down the wire screen, water, also referred to as 'white water' in the industry, is drained away and recirculated or reused in the system. As provided above, the low MD/CD TSI ratio of the media is achieved in part by increasing random fiber orientations in the paper base at the expense of fibers oriented in the machine direction (MD) during forming a paper web of the fiber mixture.

In some examples, the jet-to-wire speed ratio impacts fiber orientations and formation of the paper web or sheet. A velocity at which the jet of pulp stock is emitted from the headbox or slice of the paper making machine relative to the speed of the wire screen determines 'rush' or 'drag'. For example, a jet velocity that is slower than the wire speed produces 'drag' and a jet velocity that is faster than the wire speed produces 'rush'. When the differential between the jet velocity and the wire speed is large, then a substantial amount of the fibers of the paper web will be aligned in the machine direction (MD). However, when the differential between the jet velocity and the wire speed decreases, the fiber orientation in the MD will decrease and random fiber orientations will increase in the paper base. Depending on the paper making machine used, a jet-to-wire speed ratio of between about 0.95 and about 1.05 increases random fiber orientations (i.e., less fibers oriented or aligned in the machine direction in the paper web). For example, a jet-to-wire speed ratio of about 1 may provide a low MD/CD TSI ratio, depending on the machine configuration.

The degree of fiber orientation or alignment effects paper attributes since the fibers have different physical properties in an axial direction and a radial direction of the fibers. Less fiber orientation or alignment in the MD facilitates cross-machine direction (CD) strength to increase at the expense of the MD strength. Such higher CD strength provides for a lower MD/CD TSI ratio and a resultant paper sheet that has increased dimensional stability to reduce mis-registration during high speed printing using an inkjet web press, for example. Moreover, as the dimensional stability of the paper web increases, tendencies of the paper to curl, cockle, wrinkle and crease are reduced. Theoretically, at a jet-to-wire speed ratio of about 1.0, the MD tensile strength is at a minimum and the CD tensile strength is at a maximum (with minimum

fiber orientation). As such, the MD/CD TSI ratio of the paper web may be considered to be at its lowest achievable value at the jet-to-wire speed ratio of about 1.0, for example, and the actual ratio depends on the paper making machine and its configuration.

The method 200) of making media further comprises removing 230) water from the initial paper web in a manner that prepares the paper web for surface sizing. For example, the initial paper web is squeezed between large rollers of the paper making machine to remove most of the remaining water and form a semi-dry web. Moreover, the large rollers ensure smoothness of the paper web and uniform thickness of the paper web. To further prepare the paper web for surface sizing or coating, the semi-dry web is run through heated dryer rollers that remove more remaining water. The percent solids (%) in the paper web goes from about 0.5% at the headbox to about 95% before surface sizing and applying the outermost coating layers, such as the image receiving layer coating.

The method 200) of making media further comprises coating 240) the paper web on one or both opposite sides. For example, coating 240) the paper web comprises applying an image receiving composition that is compatible for images printed with water-based or solvent-based inkjet inks. In some examples, coating 240) the paper web may further include other intermediate coating layers (e.g., surface sizing, coatings) prior to applying the image receiving composition on the paper web.

The image receiving composition may be applied to the paper web using one or more techniques including, but not limited to, size press coating, metered size press coating, puddle size press coating, slot die coating, curtain coating, blade coating, Meyer rod coating, spray coating, dip coating, cascade coating, roll coating, gravure coating, air knife coating, cast coating, and calender stack. In some examples, the image receiving composition is applied using an inline size press or coating station with the paper making machine, during one or both of a surface sizing stage and coating stage of manufacture, for example. In some examples, the image receiving coating may replace an intermediate coating of surface sizing.

The method 200) of making media further comprises calendering 250) the coated paper web inline or offline to form the media. A calendering process may be performed after the image receiving layer is dried to improve surface smoothness and gloss, for example. The calendering process may include hardnip calender, super calender or hot soft nip calender. In some examples, smoothness and gloss target values may be achieved using an on-line hardnip or hot soft calender with the paper machine. The media is wound into large rolls that can be slit and rewound into roll sizes compatible for use in digital high speed inkjet web press printing, and may be wrapped for protection during shipping. The media made according to the method 200) described herein has an MD/CD TSI ratio of less than 2.0 and a CD residual TEA index that is greater than 300 J/Kg to facilitate digital high speed inkjet web press printing and finishing inline or offline. The media rolls may be used to produce print materials, e.g., books, magazines, newsprints, and brochures, with high print and finish quality and low production costs.

In some examples, the paper base of the media according to the principles described herein has a TEA Index greater than about 600 J/Kg, or equal to or greater than about 700 J/Kg. In some examples, the paper base has a CD TEA Index greater than about 500 J/Kg, or greater than about 800 J/Kg, or greater than about 1000 J/Kg, or equal to about 1200 J/Kg. In some examples, the paper base has a residual TEA Index greater than about 400 J/Kg, or greater than about 500 J/Kg,

or equal to or greater than about 600 J/Kg. In some examples, the paper base has a CD residual TEA Index greater than about 700 J/Kg, or greater than about 850 J/Kg, or equal to about 1000 J/Kg. Moreover in these examples, the media 5 according to the principles described herein has a CD TEA Index greater than 700 J/Kg, or greater than about 800 J/Kg, or greater than about 900 J/Kg, or equal to about 1000 J/Kg. In some examples, the media has a MD TEA Index greater than 600 J/Kg. In some examples, the media has a MD residual TEA Index greater than about 60 J/Kg, or greater than about 70 J/Kg. In some examples, the media has a CD residual TEA Index greater than 300 J/Kg and less than about 500 J/Kg.

15 In some examples, the paper base of the media according to the principles described herein has a TEA Index within a range of greater than 500 J/Kg to about 1200 J/Kg. In some examples, the paper base has a residual TEA Index within a range of about 400 J/Kg to about 1000 J/Kg. Moreover in these examples, the media according to the principles described herein has a CD TEA Index within a range of greater than 700 J/Kg to about 1000 J/Kg. In some examples, the media has a MD residual TEA Index within a range of greater than about 60 J/Kg to about 80 J/Kg. In some 20 examples, the media has a CD residual TEA Index within a range of greater than about 300 J/Kg to about 485 J/Kg.

## EXAMPLES

30 All measured values are within measurement tolerance for the equipment used, unless otherwise indicated.

Paper Base Media Samples: Paper media was fabricated using 100 parts of a fiber mixture that included about 31 parts softwood bleached kraft pulp, 25 parts hardwood bleached 35 kraft pulp, 17 parts hardwood bleached chemi-thermomechanical (BCTMP) pulp and 27 parts recycled fibers and machine broke, together in water. Both softwood and hardwood kraft pulps were refined separately using a double disc refiner to achieve target tensile stiffness and target tensile 40 energy absorption and mixed with other fibers in the ratio mentioned above. Internal cationic starch Sta-Lok® 300 was added at a dosage rate of 1.15% of the fiber weight to the fiber furnish to further increase the strength of the paper. Additionally Omya-fil® GCC inorganic filler was added into the fiber 45 furnish to achieve about 11% target ash content (measured inline) to enhance opacity, brightness and whiteness. Internal sizing agent ASA was emulsified using cationic starch at 1 to 4 ratio and added at a total dosage rate of 0.64% of the fiber weight to the fiber furnish. Additionally, other additives such as OBA and dyes for color adjustments, retention/drainage aids and biocides for operational efficiency were added into the final stock.

The paper base media was made using a commercial Fourdrinier paper machine. A very low consistency (0.5%) pulp 55 stock was jetted from the headbox at a jet-to-wire speed ratio of 1.01, and then the water was removed by filtration, pressing and drying to continuously form a web of paper base. The initial web was drained of water and passed through large rollers to remove more water and ensure smoothness and 60 uniform thickness of the semi-dry paper web. The semi-dry paper web was run through steam heated dryers of the paper making machine to remove the remaining water and achieved the final moisture target of 4.7% in the paper web (i.e., paper base media). A 'Base Only' paper media sample was created from the paper web. Moreover, a 'Coated' paper media sample was created from the paper web, as described further 65 below.

## 11

Image Receiving Layer Composition: An image receiving composition was prepared that included the following materials and amounts:

| Image Receiving Composition - Ingredients: | Parts   |
|--------------------------------------------|---------|
| HYDRAGLOSS ® 91 (kaolin clay)              | 38.3    |
| KAOCAL (calcined clay)                     | 25.6    |
| NUCLAY ® (pigment)                         | 35.9    |
| KURARAY PVA-403                            | 7.03    |
| AC-22 Dispersant                           | 0.35    |
| STR-5401 Latex                             | 1.93    |
| Calcium Chloride                           | 12.75   |
| Boric Acid Solution                        | 0.58    |
| LEUCOPHOR T-100 (OBA)                      | 0.15    |
| CARTAREN VIOLET (organic pigment)          | 0.00245 |
| STEROCOLL 802 (rheology modifier)          | 0.5     |

The image receiving composition had the following properties:

| Image Receiving Composition Fluid Properties:  |      |
|------------------------------------------------|------|
| Solid Content, %                               | 41.7 |
| pH                                             | 4.82 |
| Temperature (Deg C.)                           | 30.5 |
| Brookfield Viscosity (cP), Spindle#4 & 100 rpm | 1110 |

An offline metering size press was used to apply the image receiving composition to the paper media. Both sides of the paper media were coated with the image receiving composi-

5  
10  
15  
20  
25  
30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005  
8010  
8015  
8020  
8025  
8030  
8035  
8040  
8045  
8050  
8055  
8060  
8065  
8070  
8075  
8080  
8085  
8090  
8095  
8100  
8105  
8110  
8115  
8120  
8125  
8130  
8135  
8140  
8145  
8150  
8155  
8160  
8165  
8170  
8175  
8180  
8185  
8190  
8195  
8200  
8205  
8210  
8215  
8220  
8225  
8230  
8235  
8240  
8245  
8250  
8255  
8260  
8265  
8270  
8275  
8280  
8285  
8290  
8295  
8300  
8305  
8310  
8315  
8320  
8325  
8330  
8335  
8340  
8345  
8350  
8355  
8360  
8365  
8370  
8375  
8380  
8385  
8390  
8395  
8400  
8405  
8410  
8415  
8420  
8425  
8430  
8435  
8440  
8445  
8450  
8455  
8460  
8465  
8470  
8475  
8480  
8485  
8490  
8495  
8500  
8505  
8510  
8515  
8520  
8525  
8530  
8535  
8540  
8545  
8550  
8555  
8560  
8565  
8570  
8575  
8580  
8585  
8590  
8595  
8600  
8605  
8610  
8615  
8620  
8625  
8630  
8635  
8640  
8645  
8650  
8655  
8660  
8665  
8670<br

TAPPI method T-555. A Tensile Stiffness Index (TSI) (i.e., MD/CD ratio) was determined using a Lorentzen & Wettre TSO device (commonly described as L&W TSO tester). It used an ultrasonic method to more accurately measure this property non-destructively. The Tensile Energy Absorption (TEA) was determined for the machine direction (MD) and the cross-machine direction (CD) of each sample using an Instron Tester and a 2.54 centimeter (cm) wide strip, 100 mm gauge length, according to TAPPI method T-494. From the measured TEA, a TEA Index (TEA per basis weight) in J/Kg for the MD and the CD of the different samples were calculated. In addition, Residual Tensile Energy Absorption (TEA) Indices (in J/Kg) for the samples in the MD and the CD were also determined. Residual TEA of the samples was measured using Instron Tensile tester after high temperature conditioning and folding of the paper sample to estimate the loss in tensile energy absorption and to replicate the high temperature drying after printing and folding in the finishing. A 2.54 cm wide strip of paper was conditioned at 150° C. for 7 minutes in an oven and folded with a bow by applying 1.81 Kg weight back and forth.

TABLE 3

| Sample                    | Tensile Stiffness Index (MD/CD Ratio) | Tensile Energy Absorption Index (J/Kg) |      | Residual Tensile Energy Absorption Index (J/Kg) |      |
|---------------------------|---------------------------------------|----------------------------------------|------|-------------------------------------------------|------|
|                           |                                       | MD                                     | CD   | MD                                              | CD   |
| Control Media (Base Only) | 2.47                                  | 493                                    | 418  | 308                                             | 292  |
| New Media (Base Only)     | 1.95                                  | 712                                    | 1291 | 660                                             | 1036 |
| Control Media (Coated)    | 2.25                                  | 586                                    | 687  | 49                                              | 257  |
| New Media (Coated)        | 1.89                                  | 682                                    | 1087 | 80                                              | 484  |

TABLE 4

| Properties                      | Test Methods                              |
|---------------------------------|-------------------------------------------|
| Basis Wt                        | T-410, TAPPI Method                       |
| Caliper                         | T-411, TAPPI Method                       |
| Bulk                            | Ratio of caliper (microns)/Basis wt (gsm) |
| Opacity                         | T-425, TAPPI Method                       |
| Brightness                      | T-452, TAPPI Method                       |
| Gloss                           | T-480, TAPPI Method                       |
| Whiteness                       | CIE Ganz 82 Test Method                   |
| Smoothness (Hagerty)            | T-538, TAPPI Method                       |
| PPS Porosity                    | T-555, TAPPI Method                       |
| TEA (Tensile Energy Absorption) | T-494, TAPPI Method                       |
| HST (Hercules Sizing Test)      | T-530, TAPPI Method                       |
| Cobb                            | T-441, TAPPI Method                       |

Table 3 illustrates that the Tensile Stiffness Index (MD/CD ratio) is less than 2.0 for both the New Media (Base Only) sample and the New Media (Coated) sample, while for both of the Control Media counterparts, the MD/CD TSI ratios are both greater than 2.2. In addition, the MD/CD TSI ratio is less than 1.9 for the New Media (Coated) sample. The lower values achieved for the Tensile Stiffness Index for the New Media samples according to the principles described herein mean more random fiber orientations were achieved in the paper base. The low MD/CD ratio facilitates less CD hydro-expansion of the fibers which in turn leads to less cockle and less mis-registration and/or alignment issues during high speed web press printing with inkjet inks.

Further from Table 3, the TEA indexes of both the New Media (Base Only) and the New Media (Coated) were greater than 650 J/Kg in both the MD and CD. Moreover, both the MD and CD TEA indexes of the New Media (Base Only) were equal to or greater than about 700 J/Kg, while for the Control Media (Base Only), both the MD and CD TEA indexes were less than 500 J/Kg. In addition, the CD TEA indexes of both the New Media (Base Only) and the New Media (Coated) were greater than 1,000 J/Kg, while for the Control Media counterparts, the CD TEA indexes were less than 700 J/Kg. In fact, the respective MD and CD TEA Indexes for the New Media samples were each greater than the corresponding Control Media samples. For example, the CD TEA index of the New Media (Base Only) was about triple the Control Media (Base Only) index value. TEA predicts the durability of the media sheet under dynamic stress/work required to break the sheet, for example. These high tensile values for the New Media samples according to the principles described herein facilitate improved runnability during printing and during finishing with reduced tendency of web breaks, wrinkling, and creasing of the media.

With respect to residual TEA indexes for both MD and CD, the index values of New Media (Base Only) were at least double the values obtained from the Control Media (Base Only). In fact, the CD residual TEA index of the New Media (Base Only) was at least triple the Control Media (Base Only) index value. For the coated media, the residual TEA index values for the New Media (Coated) were almost double the values obtained for the Control Media (Coated). Higher residual strength of the sample translates into better runnability and finishing of the paper media. The residual TEA index results in Table 3 correlate well with observed improved runnability and finishing results described below.

## Runnability/Finishing

The sample Media were used to produce book signatures with a Sigma Folder manufactured by Mueller Martini with a 76.2 centimeter unwinder and B200 Sigma Collator. Finishing quality parameters such as throughput with respect to paper jams, creasing and cut quality were observed. The runnability of the Control Media (Coated) sample through the finisher exhibited one or more of paper jams, creasing and cross-cutting issues. Cut paper edges of the Control Media were frayed and unacceptable for commercial high throughput applications such as books, magazines, newsprint, and brochures. In contrast, the New Media (Coated) sample was runnable through the finisher with no problems exhibited. For example, runnability of the New Media (Coated) sample up to 450 millimeter cut length with excellent cut quality and finishing were observed. As mentioned above, the residual TEA index values in Table 3 correlated with these results. The Control Media (Coated) sample simply lacked the residual TEA strength, especially residual CD strength, to perform acceptably during runnability and finishing.

Thus, there have been described examples of a paper media used in digital high speed inkjet web press printing and a method of making the same that has a MD/CD tensile stiffness index ratio that is less than 2.0, tensile energy absorption index greater than 500 J/Kg and a CD residual TEA index greater than 400 J/Kg. It should be understood that the above-described examples are merely illustrative of some of the many specific examples that represent the principles of what is claimed. Clearly, those skilled in the art can readily devise numerous other arrangements without departing from the scope defined by the following claims.

## What is claimed is:

1. A media used in digital high speed inkjet web press printing, the media comprising:

**15**

a paper base having a MD/CD tensile stiffness index ratio less than 2.0 and a tensile energy absorption index greater than 500 J/Kg, the paper base comprising:  
 a mixture of fibers having a ratio of softwood to hard-  
 wood fibers within a range of 3 to 7 to 7 to 1; 5  
 an internal starch having a ratio of cationic starch to fiber  
 greater than 1.0%; and  
 a filler within a range of about 1.0% to about 12.0% of  
 paper base weight; and  
 an image receiving layer on a side of the paper base, 10  
 wherein the media has a CD residual tensile energy  
 absorption index greater than 300 J/Kg.  
 2. The media of claim 1, wherein the media has a basis  
 weight that is less than or equal to about 75 grams per square  
 meter. 15  
 3. The media of claim 1, wherein the cationic starch to fiber  
 ratio is within a range of 1.10% to about 5.0%.  
 4. The media of claim 1, wherein an amount of the internal  
 starch is within a range of 1.10% to about 11% of fiber weight.  
 5. The media of claim 1, wherein the fiber mixture com-  
 prises a range of about 25% to about 35% softwood chemical  
 pulp, a range of about 20% to about 30% hardwood chemical  
 pulp, and a combined amount in a range of 0% to about 50%  
 mechanical pulp, a hybrid pulp and recycled pulp, wherein a  
 total amount of softwood in the fiber mixture is at least 30%. 20  
 6. The media of claim 1, wherein the fiber mixture com-  
 prises about 30% softwood chemical pulp, about 25% hard-  
 wood chemical pulp, about 18% hybrid pulp and about 25%  
 recycled pulp, such that a total amount of softwood in the fiber  
 mixture is greater than 30%. 25  
 7. The media of claim 1, wherein one or both of up to about  
 15% of the fiber mixture is recycled pulp and up to about 10%  
 of the fiber mixture is one or both of mechanical pulp and a  
 hybrid pulp. 30  
 8. The media of claim 1, wherein the ratio of softwood to  
 hardwood fibers comprises a ratio of softwood kraft pulp to  
 hardwood kraft pulp of about 6 to about 5. 35  
 9. The media of claim 1, wherein the paper base has a MD  
 residual tensile energy absorption index and a CD residual  
 tensile energy absorption index that are each greater than 500  
 J/Kg. 40  
 10. The media of claim 1, wherein the paper base and the  
 media each has a CD tensile energy absorption index that is  
 greater than 800 J/Kg.  
 11. A media used in high speed inkjet web press printing, 45  
 the media comprising:

**16**

a paper base having a tensile energy absorption index  
 greater than 600 J/Kg comprising:  
 a mixture of fibers having a ratio of softwood to hard-  
 wood fibers within a range of 3 to 7 to 1 to 1;  
 an internal starch having a ratio of cationic starch to fiber  
 within a range of greater than 1.0% to about 5.0%;  
 a filler in an amount sufficient to achieve less than about  
 12.0% ash content; and  
 one or more agents and additives in a combined amount  
 within a range of about 0.0075% to about 9.0% of  
 fiber weight; and  
 an ink receiving layer on both sides of the paper base,  
 wherein each of the media and the paper base has a MD/CD  
 tensile stiffness index ratio of less than 2.0 and CD  
 tensile energy absorption index greater than 800 J/Kg. 15  
 12. The media of claim 11, wherein the fiber mixture fur-  
 ther comprises one or more of recycled pulp, hybrid pulp and  
 mechanical pulp in an amount independently within a range  
 of about 10% to about 30%.  
 13. The media of claim 11, wherein the paper base has a  
 residual tensile energy absorption index equal to or greater  
 than 600 J/Kg. 20  
 14. The media of claim 11, wherein the media has a MD  
 residual tensile energy absorption (TEA) index greater than  
 60 J/Kg and a CD residual TEA index greater than 300 J/Kg.  
 15. A method of making media for high speed inkjet web  
 press printing, the method comprising:  
 forming a pulp stock comprising a ratio of softwood fiber to  
 hardwood fiber ranging from 3 to 7 to 7 to 1, an internal  
 starch having cationic starch to fiber ratio greater than  
 1.0%, and a filler ranging from about 1.0% to about 12%  
 by weight of the pulp stock;  
 jetting the pulp stock onto a moving wire screen at a jet-  
 to-wire speed ratio of about 1.0 to form an initial paper  
 web; 30  
 removing water from the initial paper web in a manner that  
 prepares the paper web for surface sizing and coating,  
 the paper web having a tensile energy absorption index  
 greater than 500 J/Kg and an MD/CD tensile stiffness  
 index ratio of less than 2.0;  
 coating the paper web on one or both sides with an image  
 receiving layer; and  
 calendering the coated paper web to form the media,  
 wherein the media has a CD residual tensile energy  
 absorption index greater than 300 J/Kg. 35  
 40

\* \* \* \* \*